

June 12, 1928.

1,672,999

P. EYERMANN

## PROCESS OF PRODUCING AND PREPARING INGOTS FOR WORKING

Original Filed Dec. 15, 1923 . 2 Sheets-Sheet 1



## INVENTOR

P. Eyermann  
BY  
John Morgan  
ATTORNEY

June 12, 1928.

1,672,999

P. EYERMANN

## PROCESS OF PRODUCING AND PREPARING INGOTS FOR WORKING

Original Filed Dec. 15, 1923 2 Sheets-Sheet 2

۷۲۹



FIG 6.



**INVENTOR**

INVENTOR  
P. Egermann  
BY  
Donald Morgan  
ATTORNEY

Patented June 12, 1928.

1,672,999

# UNITED STATES PATENT OFFICE.

PETER EYERMANN, OF VIENNA, AUSTRIA, ASSIGNOR TO MAJOR I. McCREIGHT, OF DU BOIS, PENNSYLVANIA, AND REMBRANDT PEALE, JR., OF ST. BENEDICT, PENNSYLVANIA.

## PROCESS OF PRODUCING AND PREPARING INGOTS FOR WORKING.

Original application filed December 15, 1923, Serial No. 680,844. Divided and this application filed January 9, 1925. Serial No. 1,451.

The invention relates to a novel process for producing and preparing metal ingots for working.

The present invention is directed, broadly speaking, to increasing the output of finished product from a given quantity of ingots, billets, or the like, in steel and other metal working establishments; and more particularly it is directed to casting ingots, or other like units, in such form that the impurities contained in the fluent metal, or imperfections due to the pouring or casting, are thrown or deposited in certain or specific extraneous portions of the ingot and to then removing the undesirable or imperfect portions of the ingot together with a practical minimum of metal from the ingot. The invention is further directed to producing a controller for the cutting or other equivalent metal removing operation, and to a mechanism cooperating with the controlling for the purpose stated.

This application is a division of my co-pending application, Serial No. 680,844, filed December 15, 1923.

In the drawings, illustrating one apparatus for carrying out the process:

Fig. 1 is a perspective of one preferred form of metal ingots;

Fig. 2 is a section taken on line 2—2 of Fig. 1;

Fig. 3 is an illustrative diagram showing one form of rough and finished ingot;

Fig. 4 is a top plan of a lathe mechanism adapted for use in carrying out one step of the invention;

Fig. 5 is a side elevation looking at Fig. 1 from the bottom of the sheet; and

Fig. 6 is a partial elevation looking at Figs. 2 and 3 from the left on line 6—6 of Fig. 5.

It is known in metallurgical industry that non-cylindrical ingots possess valuable practical advantages over cylindrical ingots, except possibly in some narrow classes of special work. The term "non-cylindrical" as applied to ingots, billets, and the like, will be understood as including not only four-sided shapes, but others including those having several faces and edges, the later usually rounded, and having both angular and elliptical or irregular sections. The term may be further applied to ingots and billets

wherein the sides are not necessarily flat or straight, but may be either concave or convex, or the general form of the ingot or billet may be conical or otherwise tapered.

In the general practice in the art ingots or billets of these various forms have been rolled or otherwise worked up in their original shape, that is, to say, they are rolled, pressed, or forged without special preparation; and especially this is so with respect to any endeavor to preliminarily remove or eliminate the impurities existent in the fluent metal or arising from the pouring or casting of the fluent metal into the ingot or other form.

Certain preparatory work upon ingots and billets has been either suggested or practiced, but with objectives other than those of any invention and without realizing the advantages and results thereof. As an example, for the purpose of avoiding formation of seams by undue stresses in the rolled product during rolling, the ingot or billet would be shaped or planed beforehand, preparatory to rolling, to a preliminary form of such section or sections as would be the same as or similar to a finished mill product.

It has also been suggested or practiced, in order to eliminate surface defects, in products rolled from cylindrical or like ingots, to turn them on lathes before rolling, and it has also been proposed, at least, that such ingots while still warm or red hot should be milled or otherwise cut to cylindrical or analogous intermediate shapes, preparatory to being rolled.

The first mentioned of these two processes aims only to avoid the formation of seams by reducing strains and stresses during the rolling, but usually fails to attain this result in a satisfactory way.

The second of these processes effects no increase in percentage of the useful or available weight of finished rolled product, as through the milling of the ingots in a red-hot condition the location of the defects in the ingots are obliterated or covered over, and thereby an effective examination of the ingot or billet as regards its purity and freedom from defects, which is a primary condition for the increase of output aimed at, is rendered impossible. The mere turning

of cylindrical, or analogous ingots, is primarily available for very few qualities of steel and these are very limited in commercial use, and there is also a practical limit to the weight of such ingots or other kinds or qualities of products.

With reference to the importance of the present invention, it should be borne in mind that the percentage of perfect finished product hitherto obtained from even non-cylindrical raw material is comparatively low. In most mills or factories, and especially for high quality steel and other metal work, the inspections at the different stages 10 from the original ingot or billet up to the completion of the finished product, are exceedingly rigorous and thorough, during the various steps or processes of manufacturing, and there is consequently a relatively very 15 high percentage of rejections as defects are rendered apparent during the various sequential steps and processes. There is consequently but a very small percentage of the original pieces which are passed for the final 20 product. For these reasons, manufacturers have accepted and used to a certain extent cylindrical or analogous shapings, because these could be machined on ordinary lathes, and thereby the advantages of the non-cylindrical ingots were lost notwithstanding that this latter form is otherwise preferred, having other and further advantages of numerous kinds which are generally known to steel 25 manufacturers.

30 By the present invention, it is possible to use the non-cylindrical ingots and to remove the larger proportion, and practically to eliminate, impurities and defects by cutting or otherwise removing the exterior impurity 35 bearing parts. Great advantages are also realized in the matter of the weight of the ingots and the general handling of the work, in the mills or shops throughout. This goes back even so far as the open hearth or 40 crucible furnace, or the like, influencing the chemical analysis of the charge or heat.

45 By my invention the non-cylindrical ingots and billets are worked, preferably in a cold state so that practically all the impurities are cut away or otherwise removed while removing the minimum of metal from the ingot or billet. More in detail the ingots or billets are worked up to such an extent in a cold state into similarly shaped 50 but not geometrically similar non-cylindrical intermediate products. The most advantageous cross-section for such intermediate machined product is one which is similar either to the section of the raw ingot, billet 55 or the like, or to the section of the rolled or forged product, but not geometrically similar.

60 More in detail, by actual observation and experience, it is found when casting non-circular, four or more sided ingots, or equiva-

lent shapes, that slag impurities, blow holes, scales and scars are mostly located at those points or corners in the ingot which are farthest away from the center or longitudinal axis of the ingot. All such ingots, therefore, show at these corner portions the most and the deepest reaching quantity of impurities and faults, as compared with the intervening side portions of the ingot. When ingots of this kind are exteriorly cut away, or equivalently treated, so that the corner or edge portions farthest from the center or axis of the ingot are more deeply or completely removed than the intervening side surfaces (lying nearer the center or the axis), practically all of the impurities and defects are thereby removed, and this is effected with a minimum sacrifice of sound or good metal.

65 This is preferably done by automatically machining the ingot in a cold state on a lathe, with rotating work or a rotating tool, and preferably with the cutting or equivalent means controlled in its operation by a controller or pattern, shaped or otherwise designed or adapted to effect the desired result.

70 It has been ascertained by actual mill experience that despite the apparent loss of weight through this cutting off or removal of material from the surface portions of the ingot, and which amount in actual practice in many cases is from three to twelve per cent, that the resulting percentage of acceptable and saleable products is very appreciably increased, and the number of rejections resulting from subsequent inspections is greatly minimized and sometimes 75 entirely eliminated.

80 On the other hand, in ingots, or the like, of cylindrical or approximately cylindrical section, the defects distribute themselves over the entire section in an unequal and unknown manner, and the deepest machining of ingots of this form consequently gives 85 no assurance of the total or satisfactory removal of defects and impurities. The practical result is, that plants which have hitherto, due to conservative conditions, adhered to the use of cylindrical ingots, or 90 which have used unmachined or untreated non-cylindrical ingots, can by my process secure an output of finished product of high quality of a greatly increased ratio over 95 previous practice. On the average in many plants, this increase will amount to from five to twenty-five per cent of finished perfect products over results secured by the old method.

100 In practical commercial metallurgical and metal work this process is carried out by automatic mechanism, which removes the impurities and defective material until the intermediate products are free therefrom, and the intermediate products are then fin- 105

ished in the usual way, as by rolling or forging.

The carrying out of the invention will, therefore, be described in connection with a mechanism adapted for this purpose, the novel features of the mechanism and of certain instrumentalities employed therewith, mainly the controlling instrumentality for the cutting means, also constituting features 10 of my invention.

In the preferred embodiment and manner of carrying out my invention, the ingot or billet is placed in a lathe wherein the work is preferably rotated past a non-rotating, 15 longitudinally traveling cutting tool, a controller controlling the position of the cutter so as to impart to the ingot or billet the desired shape whereby the impurities and defects are eliminated by a minimum re- 20 moval of metal from the ingot or billet. The present preferred embodiment of the controlling means consists of a pattern member, rotating equally or synchronously with the ingot or billet and controlling the move- 25 ment of the cutter.

Referring now in detail to an illustrative embodiment of a lathe and a controlling instrumentality in connection with carrying out the invention, a mechanism is provided 30 wherein an ingot 1 of such general cross-section as will throw or locate during the casting and cooling the greatest part of the defects and impurities into parts of the ingot or billet farthest removed from its 35 general axis, the illustrated form being four-sided.

The ingot 1, in the present preferred form of practicing the invention, is rotated in a lathe or equivalent mechanism, and for this 40 purpose is carried between a tail stock 2 mounted upon the bed 4 of the lathe, and having a centering device 5, centrally engaging the ingot 1, all of which construction may be of any standard or suitable 45 form.

The ingot is supported at its other end by a face plate 9 provided with chucks 10 engaging and holding the ingot, the shaft 8 of the face plate being journaled in a head 50 stock 11, mounted upon the bed plate 4, the shaft being provided with a pulley drive 12. This mechanism may likewise be of any convenient or suitable form.

In the embodied form of controller for 55 removing the impurity and defect containing portions from the ingot or billet or the like with the greatest economy of metal, I prefer to use a pattern ingot or billet, although other forms of controller might be employed, 60 so far as concerns the broader aspects of the invention, such as a jacquard or perforated sheet, or other suitable or standard form. As here embodied, a pattern 16 is used, which is of, or approximately of, the 65 form and shape of the prepared ingot and

is usually and preferably of similar angular form, but with the corners or edges more rounded, or of less radius, than the ingot 1, for the purposes already stated. The pattern 16 is centrally longitudinally mounted 70 on a shaft 17, having bearings 18 and 19 supported on brackets 20 and 21, mounted upon the machine frame and preferably provided also with additional supports 22 and 23, which may optionally have adjust- 75 ing devices 24 and 25.

The shaft 17 and therewith the controller 16 are rotated synchronously with the ingot or billet 1, and for this purpose a gear wheel 25, fixed on shaft 17 is in mesh with a gear wheel 26 fixed on the shaft of the face plate 9. Thus the billet 1 and the pattern 16 will rotate synchronously and symmetrically together, that is the cutter will be at the same or corresponding point on the ingot as the detector controlling the position of the cutter will have on the pattern when that form of the controller is used.

Means are provided by the invention for cutting away the external portions of the 90 ingot or billet to correspond to the shape of the controller 16, and as embodied, a cutter 30 is removably mounted in fixed position upon the carriage 31, and is held in position by suitable means, such as clamping 95 screws 32 and 33, and its immediate carrier 28 is adjustable by a hand wheel 29. The carriage is mounted upon guideways 35 disposed longitudinally on the bed plate 4, and a longitudinal feed for the carriage is provided, such as a part 36, which is internally 100 screw-threaded upon a screw shaft 37, mounted to rotate in suitable bearings upon the machine frame, and rotated in proper relation to the turning mechanism. The foregoing mechanism is preferably of any standard or suitable form for imparting the continuous and gradual longitudinal feed to the cutter 30 along the ingot or billet 1.

Means are provided for automatically 110 controlling the position of the cutter transversely or radially to conform to the shape or equivalent requirements of the controller. As embodied, a roller 42 has its shaft 43 rotatively mounted in bearings in arms 44 and 115 45 of a plate 46, upon which the tool carrier 28 is immediately mounted. The plate 46 is provided at its external end with a cross-head 49; in the ends of which are mounted, respectively, two rods 50 and 51 held in place by nuts 52 and 53, screwed on the ends of the rods, respectively. The rods are longitudinally slidably mounted in lugs 54 and 55 fixed upon the carriage frame, and at their forward ends are also longitudinally 120 slidably mounted in lugs 56 and 57 mounted upon the plate or carriage 46.

The means for resiliently pressing the roller 42 against the pattern 16 comprises 125 helical springs 59 and 60, about rods 50 and 130

51, in compression between the corresponding lugs 54 and 55 and nuts 61 and 62 screw-threaded on the rods 50 and 51. Thus the roller 42 is gradually and symmetrically fed 5 or traveled along the surface of the pattern 16, and describes thereon an endless circumferential path somewhat analogous to a helix but being non-circular due to the cross-sectional shape of the ingot and the cutter 30 is 10 positioned to cut away the ingot 1 in conformity with the indications or requirements of the controller 16.

Referring to the explanatory and exemplary diagram of Fig. 3, the exterior outline 15 *a* may be taken as representing a cross-section of the raw ingot, and the defects and impurities will be mainly if not entirely deposited in the corner or edge portions *c*. The area represented by *b* may be taken as a typical corresponding cross-section of the machined or otherwise treated billet and the intervening area between *a* and *b* will be a 20 corresponding cross-sectional representation of the removed portions of the ingot, whereby all, or practically all, of the defects and impurities will be removed, with a minimum 25 removal of the sound metal from the ingot.

It will be understood that the diagrams

and the references herein to percentages and quantities, as well as other details, are exemplary and explanatory, but are not restrictive of the invention.

The invention in its broader aspects is not limited to the details of process nor to the specific mechanisms shown and described, but departures may be made therefrom within the scope of the accompanying claim without departing from the principles of the invention and without sacrificing its chief 40 advantages.

What I claim is:—

The process of producing and preparing an ingot for working which comprises casting the ingot into a form having a polygonal cross section, with the longitudinal edges of the ingot extending substantially throughout the entire length thereof, permitting the ingot to cool, and then selectively cutting away the surface of said ingot so as to remove a minimum of sound metal 45 by cutting away substantially only the longitudinal edge portions, thus removing the greatest amount of defective metal.

In testimony whereof, I have signed my name to this specification.

PETER EYERMANN.